

3,158,450  
TRIAZINYL DERIVATIVES AS GASOLINE  
ADDITIVES

Gaetano F. D'Alelio, South Bend, Ind., assignor, by direct and mesne assignments, to Dal Mon Research Co., Cleveland, Ohio, a corporation of Delaware  
No Drawing. Filed Dec. 7, 1961, Ser. No. 157,856  
20 Claims. (Cl. 44—63)

This invention relates to improvements in gasoline-type 10 motor fuels.

To increase the anti-knock value of gasoline-type motor fuel, such fuels are modified by the addition of a tetraalkyl lead, such as tetramethyl lead or tetraethyl lead with a lesser amount of halohydrocarbon, such as an alkyl or alkylene halide, as for example, ethylene dichloride, ethylene dibromide, carbon tetrachloride, and the like. The mixture of a tetraalkyl lead and a haloalkane is known as "ethyl fluid" and is used extensively in automotive and aviation gasolines in amounts of 1 cubic centimeter to 4 or 5 cubic centimeters per gallon of gasoline.

In the modern high compression engine, even though the use of "ethyl fluid" is beneficial, its use tends to cause "surface" or "pre-ignition," which results in misfiring and disrupts the regular rhythm of engine operation. This "surface ignition" in gasoline containing lead derivatives is due to the deposition of various lead compounds within the combustion chamber of the engine, which thereafter produces hot spots or glow points in the combustion chamber, causing pre-ignition and pre-combustion.

Another adverse effect which results from the use of leaded gasoline is misfiring of the engine due to spark-plug fouling. Though the use of halohydrocarbon scavengers has only partially remedied the problems resulting from the deposition of lead compounds in the combustion chamber, it has been less effective in the prevention of spark-plug fouling, which particularly in aircraft gasoline combustion engines, is a serious problem.

It has now been found that the above disadvantages accompanying the use of leaded gasoline can be substantially minimized and even eliminated by the addition of a small amount of certain 1,3,5-triazine phosphonic acid derivatives to leaded gasoline, thereby reducing pre-ignition and spark-plug fouling to a significant degree. The additives of this invention are derivatives of 1,3,5-triazines,



represented herein as  $C_3N_3$ , to which is attached, through the carbon atoms of the triazine ring, at least one phosphonium moiety,



directly to the carbon atom,



Since the triazinyl radical is trivalent, these derivatives can contain no more than three such phosphonium groups,



The only requirement for the compounds used in the practice of this invention is that they contain at least one such phosphonium group, and thus, though the other valencies of the triazine ring may be occupied by any monovalent radical, certain advantages accrue, as hereinafter shown, when more than one phosphonium group is present, or when the other monovalent radicals are especially selected to perform a special or selected function. These triazine derivatives may also be expressed by the formula



in which  $n$  represents a numerical value of 1 to 3, A represents a radical selected from the class of



wherein B is selected from the class of oxygen and sulfur, R represents a radical selected from the class consisting of hydrogen, a hydrocarbon radical containing from one to twenty carbon atoms, the hydroxy and halogenated derivatives of said hydrocarbon radicals, M represents a metal selected from the class of alkaline and alkaline earth metals, K represents a radical selected from the class of  $-BR$ ,  $-BM$ , and  $NR_2$  (where the oxygen derivatives are to be specified K' is substituted for K), and Y represents a monovalent radical. For ordinary usage the nature of the monovalent radical Y is not critical since the effect of the phosphonium radical on the lead is not affected. For example, Y can be H,  $-R$ ,  $-BH$ ,  $Br$ ,  $-NR$ ,  $-NRNR_2$ , halogen, and the hydroxy-, halogeno-, acetoxy, alkoxy, carbamido and sulfamido derivatives of the R group such as



However, when it is desirable to impart special properties to the triazinyl phosphonium derivatives used in the practice of this invention, such as increased solubility in petroleum products, then R represents a hydrocarbon radical possessing from 5 to 20 carbon atoms. When it is desired to impart further special properties to these compounds, such as antioxidant properties, and to retain solubility in hydrocarbons, or to have these compounds act as stable halogen carriers, while considering also economic factors and availability of raw materials, then, preferably Y is  $R'$ ,  $R'B$  or  $R'_2N$  wherein  $R'$  represents radicals containing 5 to 20 carbon atoms selected from the class of R, halogenated derivatives of R and hydroxy aryl radicals such as



The hydrocarbon group represented by R include saturated or unsaturated, e.g., ethylenic or acetylenic, straight and branched chain aliphatic hydrocarbon radicals, aryl radicals, alkylaryl radicals, aralkyl radicals, saturated and unsaturated alicyclic and cyclic radicals, including spiro radicals, and the like. The halogenated hydrocarbon derivatives are the fluoro, chloro, bromo, and iodo derivatives. For economic reasons, the chloro and bromo derivatives are preferred.

The alkaline and alkaline earth metals represented by

M can be either monovalent or polyvalent, including for example, potassium, sodium, lithium, parium, calcium, cesium, magnesium, strontium, etc.

Further versatility is demonstrated in these compounds by the nature and number of the phosphonium-type groups attached to the triazine ring. When a high concentration of phosphorus is desired in the addition, then three such groups are attached to the nucleus. If the lowest concentration of carbon is desired in this compound then the methyl ester derivative,



is used, whereas if a high carbon content is desired, the higher alcohol esters are satisfactory, thus



Furthermore, if a detergent property is desired, the triazinyl phosphonium ester may be saponified to produce the mono- or di-salt, thus



If a non-ionic type detergent is desired, the phosphonic acid can be reacted with an alkylene oxide to obtain such a product, thus



wherein  $n'$  has a numerical value of 3 to 15.

The phosphonium moiety can also act as a carrier of halogen atoms, thus



It can also be a carrier of an antioxidant structure, thus



It can also serve in a joint function as a halogen carrier and antioxidant, such as in the moiety



The compounds used in the practice of this invention are prepared readily by the reaction of a halo-s-triazine with a phosphite ester as follows:



It is obvious from the foregoing that these additive compounds, because of the various reactions that can be

effected by the phosphites,  $P(OR)_3$ , with either a mono-, di-, or tri-halo triazine, can be synthesized to contain more than the phosphorus atoms as phosphates or phosphites, and therefore can perform more functions when used as an additive. Furthermore, since the phosphonium structure is attached to a triazine ring which contains nitrogen in a relatively inert form, the combustion of these compounds produces oxides of nitrogen which also assist in removal of combustion cylinder deposits.

The synthesis of typical compounds used in the practice of this invention is illustrated in the following examples. Unless specified otherwise, parts and percentages recited herein are parts and percentages by weight.

#### Example I

One hundred thirteen (113) parts of cyanuric chloride is added gradually to 575 parts of triethyl phosphite over a period of 1 hour. During the addition considerable heat is generated and some ethyl chloride is liberated. The resultant mixture is maintained at 90-105° C. for 1 hour and then allowed to cool to room temperature. The cooled mass is extracted with low boiling petroleum ether to remove excess triethyl phosphite and then recrystallized from ethyl ether. The crude yield is about 99 per cent, and the melting point of the recrystallized product is 94-95° C. Analyses show 38.36% carbon and 6.12% hydrogen, which correspond closely with the theoretical values of 36.84% carbon and 6.11% hydrogen for the compound having the formula



When other phosphites of the formula  $P(OR)_3$  and  $P(SR)_3$  are used instead of the triethyl phosphite with R representing butyl, amyl, cyclohexyl, phenyl, chlorophenyl and acetoxyphenyl, the corresponding triazine phosphonium and thiophosphonium derivatives are obtained.

#### Example II

Example I is repeated using an equivalent amount of trimethyl phosphite instead of triethyl phosphite and there is obtained



45 of melting point 124.5° C., which on analysis shows C, 26.89% and H, 4.68%, which is in good agreement with the calculated values for carbon and hydrogen.

#### Example III

Example I is repeated, using molar equivalents of tri-n-propyl phosphite instead of triethyl phosphite, and there is obtained



as an oil which slowly crystallizes on standing at 0° C.

#### Example IV

Example I is repeated using molar equivalents of tri-(beta-chloroethyl)-phosphite instead of triethyl phosphite and there is obtained



65 melting point 53-54° C., which on analysis shows 25.59% C and 3.38% H, which compares with the theoretical values of 25.86% C and 3.45% H respectively.

#### Example V

Example I is repeated using molar equivalents of tri-allyl phosphite instead of triethyl phosphite, and there is obtained



5

which on analysis and molecular weight determination give values in close agreement with the theoretical values for this compound. When the trimethylallyl phosphite is used in equivalent amount instead of the triallyl phosphite, there is obtained



*Example VI*

One hundred fifty (150) parts of



are added to 200 parts of carbon tetrabromide and 80 parts of bromine added to the mixture at 20-50° C. and there is obtained in solution in ethylene dibromide, the compound.



This solution can be used in lead gasoline as such, or the halogenated phosphonium triazine derivative isolated by removal of the carbon tetrabromide under reduced pressure. When the methylallyl derivative is used instead of the allyl derivative, there is obtained



*Example VII*

In a suitable reactor equipped with stirrer and reflux condenser a mixture of 145.5 parts of 2,4-diamino-6-monochloro-1,3,5 triazine, 200 parts of triethyl phosphite and 200 parts of benzene are refluxed for eight hours with the released ethyl chloride being allowed to escape. The reaction mass is cooled and



separated by filtration, washed with alcohol, and dried. Analysis of the product gives the following values: 34% carbon, 28.1% nitrogen, 5.35% hydrogen, and 12.2% phosphorus; these values are in close agreement with the theoretical values. When 165 parts of the corresponding monoamino-dichlorotriazine are reacted in place of the monoaminochlorotriazine with 380 parts of triethyl phosphite, an almost quantitative yield of



is obtained, which on analysis gives values of 35.16% carbon, 5.89% hydrogen, 15.35% nitrogen, and 17.21% phosphorus. These values are in close agreement with the theoretical values.

When this diester is allowed to stand at room temperature with aniline, the corresponding



is obtained.

*Example VIII*

The procedure of Example I is repeated, using trioctylphosphite in molar quantities equivalent to triethylphosphite, and there is isolated the compound



Similarly, the triesters of decyl, dodecyl, tetradecyl, and octadecyl alcohols are prepared.

*Example IX*

One hundred thirty-seven parts of 2-chloro-4,6-dihydroxy-s-triazine prepared from cyanuric chloride by the method given in J. prakt. Chem., (2), 75, 103 (1907) are reacted with 104 parts of trimethyl phosphite according

to the procedure of Example I. A quantitative yield of



is obtained. When an equivalent weight 2,4-dichloro-6-hydroxy-s-triazine is used instead of the 2-chloro-4,6-dihydroxy compound, the corresponding derivative



is obtained in quantitative yield.

When



is treated with aniline, methyl amine and diethyl amine respectively, according to the procedure of Example VII, the corresponding amides are obtained respectively,



*Example X*

Two hundred thirty-six parts of  $\text{HOC}_6\text{H}_4\text{NH}(\text{C}_3\text{N}_3)\text{Cl}_2$ , prepared according to the procedure of U.S. Patent 2,393-755, in 250 parts of benzene are refluxed ten hours with 195 parts of tri-n-propyl phosphite. Then the benzene is removed under a reduced pressure, using a water aspirator, to give a quantitative yield of crude but relatively pure



When an equivalent amount of  $(\text{HOC}_6\text{H}_4\text{NH})_2\text{C}_3\text{N}_3\text{Cl}$  (see U.S. Patent 2,393,755) is used instead of the dichloro-triazine of this example, there is obtained



Treatment of these phosphonic esters with the amines of Example IX by the procedure of Example VII produce the corresponding phosphonamides, whereas when diethyl amine or decyl amine is used, there is obtained respectively



*Example XI*

70 2-amino-4,6-dichloro-s-triazine prepared according to the method of Berichte, 32, 691 (1889), is converted to 2-amino-4-hydroxy-6-chloro-s-triazine by the hydrolysis procedure of J. prakt. Chem., (2), 75, 103 (1907). Thereafter, 136 parts of 2-amino-4-hydroxy-6-chloro-s-triazine are reacted with 250 parts of tri-n-butyl phosphite

according to the procedure of Example I, and there is obtained



Example XII

One hundred thirty-eight parts of 2-amino-4,6-dichloro-s-triazine are mixed with 250 parts of tri-secondary butyl phosphite and allowed to react in a suitable container at room temperature for twenty-four hours, and at 60° C. for 8 hours; there is obtained on recrystallization of the reaction product from acetone-water a substantial yield of



Example XIII

Two hundred and fifteen parts of 2-phenyl-4,6-dichloro-s-triazine prepared by the procedure of U.S. Patent 1,911,689 is reacted by the procedure of Example II with 210 parts of trimethyl phosphite, and there is obtained



Treatment of this product with ammonia, and aniline according to the procedure of Example VII results in



Example XIV

One hundred and nine parts of



are heated at 100° C. with 210 parts of phenol containing 1 part of magnesium oxide for 14 hours or until methanol is no longer released from the reaction. From the reaction product there is obtained



When this procedure is repeated with p-chloro phenol, 50 there is obtained



Example XV

2,4-di-o-dichlorophenyl-6-chloro-s-triazine is prepared by the method of Chem. Ztg. 36, 378 (1912), and when this product is used in the procedures of Examples VII, IX, and XIV there is obtained respectively



Example XVI

Cyanuric chloride is converted to 2-butyl-4,6-dichloro-s-triazine by the method of U.S. Patent 1,911,689, and thereafter converted to 2-butyl, 4-chloro-6-thiocarbamyl-methyl sulfide,  $(C_4H_9)(NH_2OCCH_2S)-(C_3N_3)Cl$ , by the methods given in U.S. Patent 2,295,562.

The reaction of this product according to the procedure of Example II with triamyl phosphite yields the compound



Example XVII

Thirty parts of



10 parts of 37.1%  $CH_2O$  aqueous solution and 0.1 part of NaOH are mixed and allowed to stand 48 hours at room temperature, or until substantially all of the formaldehyde has disappeared and there is obtained a dispersion in water of the compound.



The addition of 4.5 parts of dimethyl amine or 7 parts of diethyl amine to this compound at room temperature produces, respectively,



Example XVIII

Two hundred ten parts of



40 165 parts of 37% formaldehyde aqueous solution, and 3 parts of KOH are allowed to stand at room temperature with constant agitation for 48 hours, or until substantially all of the formaldehyde has disappeared and there is obtained a dispersion of the compound



which is dried in a vacuum at room temperature.

Example XIX

Two hundred parts of 2,4-di-ethylamino-6-chloro-s-triazine prepared by the method of JACS 73, 2982 (1951) is reacted with 155 parts of triethyl phosphite as in the procedure of Example II, and there is obtained the compound



When 203 parts of  $P(SC_2H_5)_3$  are substituted for the 60  $P(OC_2H_5)_3$  of this example the corresponding compound,



65 is obtained, which when reacted with aniline according to the procedure of Example I, yields



With p-aminophenol, it gives



9

## Example XX

2-dimethylamino-4,6-dichloro-s-triazine is prepared according to the procedure of JACS 73, 2982 (1951) and converted to the 4-thiocarbamyl methyl sulfide,



by the method given in U.S. Patent 2,295,562. This is reacted with triethyl phosphite by the procedure of Example IX to give



## Example XXI

2-chloro-4,6-dimethoxy-s-triazine is prepared according to the procedure of JACS 73, 2989 (1951) and reacted with one molar equivalent of triallyl phosphite according to the procedure of Example I yields



## Example XXII

2,4-dichloro-6-methoxy-s-triazine is prepared according to the procedure of JACS 73, 2989 (1951) and reacted with two molar equivalents of trimethyl phosphite by the procedure of Example I to give



Substitution of 2,4-dichloro-6-phenoxy-s-triazine for the corresponding methoxy derivative in this example produces



## Example XXIII

Sulfanilamide is reacted with cyanuric chloride 2,4-dichloro-6-(4-sulfamoylanilino)-s-triazine according to the method of J. Org. Chem., 24, 643 (1959), and when this compound is reacted with two molar equivalents of triethyl phosphite according to the procedure of Example II, there is obtained the compound



When 2-chloro-4,6-di-(4-sulfamoylanilino)-s-triazine is used instead of the above dichloro-compound with at least one molar equivalent of triethyl phosphite, there is obtained instead



when a-amino-4-chloro-6-(4-sulfamoylanilino)-s-triazine is used instead of the dichloro compound, then, there is obtained



## Example XXIV

2-ethyl-4,6-dichloro-s-triazine is prepared according to the method of U.S. Patent 1,911,689 and converted by reaction with ethyl aminocaproate by the method of U.S. Patent 2,328,961 to



When reacted with one molar equivalent of tribenzyl phosphate by the procedure of Example II produces



## Example XXV

Equivalent quantities of 2,4-dichloro-6-(2-hydroxyeth-

10

ylamino)-s-triazine are substituted for the dichloro-triazine of Example XV and there is obtained a good yield of



When the 2-chloro-4,6-di-(2-hydroxyethylamino)-s-triazine is used with one molar equivalent of the phosphite, there is obtained.



## Example XXVI

2,4-dichloro-6-(beta-cyanoethyl sulfide)-s-triazine is prepared by the method of U.S. Patent 2,295,561 and is treated with two molar equivalent of tri-cyclohexyl phosphite by the procedure of Example II and there is obtained



When the above cyanoethyl sulfide derivative is replaced by an equivalent molar quantity of 6-carbanyl-methyl sulfide prepared by the procedure of U.S. Patent 2,295,562, there is obtained



## Example XXVII

2,4-dichloro-6-semicarbazido-s-triazine is prepared by the method of U.S. Patent 2,295,565 and treated with two molar equivalent of tridecyl phosphite according to the procedure of Example II and there is obtained



## Example XXVIII

2,4-dichloro-6-ureido-s-triazine is prepared according to the method of U.S. Patent 2,295,563 and reacted with tripropyl phosphite by the procedure of Example II and there is obtained



## Example XXIX

2,4-dichloro-6-(p-sulfamyl-phenyl - carbamyl - methyl sulfide) is prepared according to the method of U.S. 2,316,692 and reacted with tri-(p-bromobenzyl) phosphite by the procedure of Example II and then is obtained



## Example XXX

2,4-dichloro-6-amino-s-triazine is converted to 2-para-hydroxyphenylcarbamyl methyl sulfide by reaction with  $\text{HSCH}_2\text{CONHC}_6\text{H}_4\text{OH}$  by the procedure of U.S. Patent 2,295,562 and when this product is reacted according to the method of Example II, with triethyl phosphite, there is obtained



## Example XXXI

Cyanuric chloride is converted to 2,4-dichloro-6-phenyl-s-triazine by the method of U.S. Patent 1,911,689 and by reaction with para-hydroxy benzamide (by the procedure used for  $\text{HSCR}_2\text{CONH}_2$  type compound in U.S. Patent 2,295,562) is converted to



which when reacted with triethyl phosphite according to the procedure of Example II produces



11  
Example XXXII

2,4-di-octadecylamino-6-monochloro-s-triazine is prepared by the method given in JACS 73, 2982 (1951) and reacted with a molar equivalent of trimethyl phosphite by the procedure of Example II, and the product isolated as



which when saponified by refluxing with methanolic 10 NaOH is converted to



which is water-dispersible as wetting agent, emulsifier or 15 detergent.

If the procedure of this example is repeated using 2,4-dichloro-6-octadecylamino-s-triazine prepared by the method of JACS 73, 2982 (1951) and reacted with two molar equivalent of trimethyl phosphite, there is obtained



which is a more effective dispersing agent than the mono-compounds. This same behavior is observed in the lower alkyl derivatives containing a total of at least 10 25 carbon atoms in the aliphatic chain, thus



The free acid is readily liberated from these salts by treatment with excess quantities of strong inorganic acids such as sulfuric or phosphoric acid. The free acids are 35 useful as rust inhibitors and pickling agents, and have the formula



and



respectively.

Other metal salts such as potassium, lithium, calcium, magnesium, silver, copper, titanium, zirconium, molybdenum, etc., such as those known metals which form both inorganic or organic salts can be prepared by the known metathesis reactions or by treatment of reaction of the oxides or hydroxides of such metals with the free s-triazine phosphonic acids.

## Example XXXIII

Cyanuric chloride is converted to 2,4-dimercapto-6-chloro-s-triazine by the method of J. prakt. Chem. (2), 34, 152 (1886), and when this compound is reacted with molar equivalents of trimethyl phosphite according to the procedure of Example II, there is obtained



## Example XXXIV

The procedure of Example I is repeated using molar equivalents of diphenylmethyl phosphite instead of triethyl phosphite and there is obtained



The utility of the s-triazinyl phosphonium compounds used in the practice of this invention may be illustrated using gasolines of wide boiling range and with various octane ratings. A typical gasoline used as a reference

gasoline in the following tests and has the following distillation characteristic.

|          |     |
|----------|-----|
| IBP, °F. | 96  |
| 10%, °F. | 127 |
| 20%, °F. | 145 |
| 30%, °F. | 161 |
| 40%, °F. | 176 |
| 50%, °F. | 200 |
| 60%, °F. | 225 |
| 70%, °F. | 258 |
| 80%, °F. | 299 |
| 90%, °F. | 358 |
| EP, °F.  | 428 |

(Octane rating, 98.5.)

to which is added 4 cc. of tetraethyl lead per gallon of fuel, to which may be added ethylene dibromide (EDB) as a scavenger. The amount of EDB added used is expressed in the term, Theory EDB, which designates the amount of scavenger required to react stoichiometrically with all of the lead anti-detonant so that all of the lead atoms react with all of the halogen atoms to form  $\text{PbX}_2$ , and thus one theory of halogen scavenger contains two halogen atoms for each atom of lead in the lead anti-detonant.

The term "Theory S-T-P" designates the amount of s-triazinyl phosphonium compound required to react stoichiometrically with all of the lead so that all of the lead atoms and all of the phosphorus atoms to form



which may be expressed also as  $\text{Pb}(\text{PO}_4)_{2/3}$ , and thus only two phosphorus atoms are required for each three atoms of lead. Thus it may be seen that one mole of



will be 4.5 Theory S-T-P, while



will be 3 Theory S-T-P, and



45 will be 1.5 Theory S-T-P when Y does not contain a phosphonium group.

On a molar basis, improvements are noted when these phosphonium compounds are present in the ratio of as little as 0.0005, preferably at least 0.05, mole of phosphonium compound per mole of organo-lead compound. 50 Generally no added improvement is noted by using more than 3 moles of phosphonium compound per mole of organo-lead compound.

When the s-triazinyl phosphonium compounds of this 55 invention contain halogen atoms as well, then they will also have EDB theory value, thus



60 will be 3 Theory EDB and 4.5 Theory S-T-P.



will be 6 Theory EDB and 4.5 Theory S-T-P.



will be 4 Theory EDB and 3 Theory S-T-P.

Other theoretical and S-T-P values of the numerous examples given hereinabove are similarly obvious.

## Example XXXV

A suitable engine (such as defined in ASTM-D-908-55 and in ASTM-D-357-33) suitably instrumented with electrical pressure indicators and electrical ionization gap

recorders is operated with the reference gasoline described above with one (1) Theory EDB scavenger for 25 minutes of lean mixture cruising conditions followed by 5 minutes of rich mixture idling, and this ratio of 25 minutes to 5 minutes cycle repeated until spark plug fouling occurs, as evidenced by misfiring. The tests are then repeated, using different S-T-P compounds and the time for fouling to occur are observed, as summarized in Table I.

TABLE I

| S-T-P Additive                                                                                                | Theories S-T-P           | Theories EDB             | Percent Increase in misfiring time |
|---------------------------------------------------------------------------------------------------------------|--------------------------|--------------------------|------------------------------------|
| None                                                                                                          | 0                        | 1                        | 0                                  |
| $\text{C}_3\text{N}_3[\text{P}(\text{O}\text{C}_4\text{H}_9)_2]_3$                                            | 0.1<br>0.2<br>0.2<br>0.3 | 0.5<br>0.5<br>0.1<br>0.6 | 250<br>325<br>365<br>385           |
| $\text{C}_3\text{N}_3[\text{P}(\text{O}\text{C}_6\text{H}_5)_2]_3$                                            | 0.2                      | 0.8                      | 400                                |
| $\text{C}_3\text{N}_3[\text{P}(\text{O}\text{C}_6\text{H}_4\text{Cl})_2]_3$                                   | 0.2                      | 0.6                      | 450                                |
| $\text{C}_3\text{N}_3[\text{P}(\text{O}\text{CH}_2\text{CH}_2\text{Cl})_2]_3$                                 | 0.6<br>0.6               | 0<br>0.1                 | 400<br>450                         |
| $(\text{C}_3\text{N}_3)_2[\text{P}(\text{O}\text{CH}_2\text{CHBrCH}_2\text{Br})_2]_3$                         | 1.0<br>0.5<br>0.7        | 0<br>0<br>0.05           | 405<br>435<br>440                  |
| $\text{ClC}_6\text{H}_5\text{O}(\text{C}_3\text{N}_3)_2[\text{P}(\text{O}\text{C}_6\text{H}_4\text{Cl})_2]_2$ | 0.3<br>0.05              | 0.2<br>1.0               | 415<br>285                         |
| $(\text{C}_5\text{H}_{11}\text{NH})_2\text{C}_3\text{N}_3[\text{P}(\text{O}\text{O}_2\text{H}_5)_2]$          | 0.2                      | 0.8                      | 385                                |
| $(\text{C}_3\text{N}_3)_2[\text{P}(\text{O}\text{C}_3\text{H}_7)_2]_3$                                        | 0.5                      | 0.5                      | 345                                |

## Example XXXVI

The engine suitably instrumented as in the previous example to detect abnormal ignitions and pressure rises in the combustion chamber is operated with the reference gasoline containing 2.7 cubic centimeters of tetramethyl lead in the following cycles, simulating driving conditions equivalent to

- 1 hour at 60 miles per hour
- 3 hours at 30 miles per hour
- 6 hours of start and stop driving consisting of
  - 2 hours idling,
  - 2 hours accelerating to 30 miles per hour, and
  - 2 hours decelerating to idling

for a total of ten hours for the cycle, which is repeated 10 times for a total of 100 hours.

The compositions of Example XXXIV are compared in this engine under the cycle given, and all of the compositions containing S-T-P when compared with the composition containing no S-T-P and 1 Theory EDB show a very substantial decrease in the percentage of pre-ignition which result in misfirings.

It also may be seen from Table I that the S-T-P compounds can be used alone or in conjunction with halohydrocarbon scavengers.

When the preceding tests are repeated using the corresponding thiophosphonium compounds, improved results are likewise noted.

The invention claimed is:

1. A fuel consisting essentially of gasoline, a minor

amount of a tetraalkyl lead anti-detonant sufficient to impart anti-knock properties to said fuel and 0.0005-3 moles, per mole of said tetraalkyl lead anti-detonant, of a s-triazinyl phosphonium compound having at least one and no more than three phosphonium radicals attached to the carbon atoms of said s-triazinyl nucleus, said phosphonium radical being selected from the class consisting of



radicals, wherein B is an atom selected from the class consisting of oxygen and sulfur, R represents a radical selected from the class consisting of hydrogen, hydrocarbon radicals having no more than 20 carbon atoms therein, and derivatives of said hydrocarbon radicals having only derivative groups attached thereto selected from the class consisting of hydroxy and halo radicals, K represents a radical selected from the class consisting of  $-\text{BR}$ ,  $-\text{BM}$  and  $-\text{NR}_2$ , and M is a metal selected from the class consisting of alkali and alkaline earth metals.

2. A fuel consisting essentially of gasoline, a minor amount of a tetraalkyl lead anti-detonant sufficient to impart anti-knock properties to said fuel and 0.0005-3 moles, per mole of said tetraalkyl lead anti-detonant, of a s-triazinyl phosphonium compound having at least one and no more than three phosphonium radicals attached to the carbon atoms of said s-triazinyl nucleus, said phosphonium radical having the formula



35 wherein R represents a radical selected from the class consisting of hydrogen, hydrocarbon radicals having no more than 20 carbon atoms therein, and derivatives of said hydrocarbon radicals having only derivative groups attached thereto selected from the class consisting of hydroxy and halo radicals, K' represents a radical selected from the class consisting of  $-\text{OR}$ ,  $-\text{OM}$ ,  $-\text{NR}_2$ , M is a metal selected from the class consisting of alkali and alkaline earth metals.

3. A fuel of claim 2 wherein said anti-detonant is selected from the class of tetra-ethyl and tetra-methyl lead.

4. A fuel of claim 1 wherein said anti-detonant is selected from the class of tetra-methyl and tetra-ethyl lead.

5. A fuel consisting essentially of gasoline, a minor amount of a tetraalkyl lead anti-detonant sufficient to impart antiknock properties to said fuel and 0.0005-3 moles, per mole of said tetraalkyl lead anti-detonant, of a s-triazinyl phosphonium compound having at least one and no more than three phosphonium radicals attached to the carbon atoms of said s-triazinyl nucleus, said phosphonium radical having the formula



60 wherein R represents a radical selected from the class consisting of hydrogen, hydrocarbon radicals having no more than 20 carbon atoms therein, and derivatives of said hydrocarbon radicals having only derivative groups attached thereto selected from the class consisting of hydroxy and halo radicals.

6. The fuel of claim 1 in which said phosphonium compound is



7. The fuel of claim 1 in which said phosphonium compound is



8. The fuel of claim 1 in which said phosphonium compound is



15

9. A fuel of claim 8 in which said anti-detonant is selected from the class of tetra-methyl and tetra-ethyl lead.

10. A fuel of claim 1 in which said phosphonium compound is



11. A fuel of claim 10 in which said anti-detonant is selected from the class of tetra-methyl and tetra-ethyl lead.

12. A fuel of claim 1 in which said phosphonium compound is



13. A fuel of claim 12 in which said anti-detonant is selected from the class of tetra-methyl and tetra-ethyl lead.

14. The fuel of claim 1 in which said phosphonium compound is



15. A fuel of claim 14 in which said anti-detonant is selected from the class of tetra-methyl and tetra-ethyl lead.

16. The fuel of claim 1 in which said phosphonium compound is

25

20

25

16



17. The fuel of claim 1 in which said phosphonium compound is



18. The fuel of claim 1 in which said phosphonium compound is



19. The fuel of claim 1 in which said phosphonium compound is



20. The fuel of claim 1 in which said phosphonium compound is



References Cited in the file of this patent

UNITED STATES PATENTS

2,685,581 Coover \_\_\_\_\_ Aug. 3, 1954  
2,751,384 Coover et al. \_\_\_\_\_ June 19, 1956  
3,011,998 D'Alelio \_\_\_\_\_ Dec. 5, 1961

FOREIGN PATENTS

565,182 Canada \_\_\_\_\_ Oct. 28, 1958  
572,281 Canada \_\_\_\_\_ May 5, 1959